

## UNITED STATES PATENT OFFICE

2,037,331

## AIR DRYING IMITATION LEATHER FINISH

Harvey G. Kilttredge and Albert J. Turner,  
Dayton, Ohio, assignors to The Kay and  
Ess Chemical Corp., Dayton, Ohio, a cor-  
poration of Delaware

No Drawing. Application December 28, 1934,  
Serial No. 759,548

8 Claims. (Cl. 134—26)

This invention relates to enamels and var-  
nishes, and particularly to imitation leather fin-  
ishes in colors.

It is the object of the invention to produce an  
imitation leather finish that upon drying will  
have the appearance of leather, but which does  
not need to be baked at high temperatures here-  
tofore required in the art from 300 to 400 de-  
grees F. It also eliminates the use of embossing  
rolls in order to give the appearance of leather,  
because upon drying in the air at ordinary tem-  
peratures, from 60 to 70 degrees F., the material  
of the present invention gives the appearance of  
leather, and has the soft, smooth body and feel  
of leather.

It is the purpose of this invention to produce  
an imitation leather finish that will air dry at  
ordinary temperatures of from 60 to 70 de-  
grees F.

It is a further object to provide such a finish  
which does not have to be heat-treated after  
the finish has been applied prior to the baking  
operation.

It is also an object to eliminate both the heat-  
treating and baking operations.

In order to accomplish the objects of this in-  
vention we first prepare a varnish, hereafter  
known as Varnish A.

30 Varnish A

A typical formula is the following:

|                             | Pounds |
|-----------------------------|--------|
| Amberol B/S 1 Lt.           | 67     |
| Litharge                    | 3 1/2  |
| Manganese linoleate (solid) | 8 1/2  |
| Cobalt linoleate (do)       | 2      |
| Gallons                     |        |
| China-wood oil              | 20     |
| Linseed oil                 | 2 1/4  |
| Heavy petroleum naphtha     | 14     |
| Light petroleum naphtha     | 14     |

45 Amberol is a phenol, formaldehyde, synthetic  
resin. It is made as follows: one hundred parts  
of phenol aldehyde resin difficultly fusible and  
only partly soluble in benzol and other solvents  
and produced, for instance, by heating 108 parts  
of cresol with 60 to 75 parts of formaldehyde (30%  
by weight) and distilling off the water and the  
uncombined cresol, are added gradually to 800  
parts of melted colophony. The whole mixture is  
then heated in an autoclave until a resin is pro-  
duced which is clear in the cold, homogeneous  
and free from smell of phenol. The volatile sub-

stances are then removed while stirring and 100  
parts of glycerol of 28 degrees Bé. are added in  
small quantities whereupon the mixture is heat-  
ed to 250 degrees C. and kept at this tempera-  
ture for several hours while being stirred care-  
fully. A typical formula for amberol is shown in  
United States Patent No. 1,623,901.

In order to prepare this varnish, we first take  
20 gallons of China-wood oil or tung oil and 2 1/4  
gallons refined linseed oil. These oils are mixed 10  
and heated at a normal rate to 480 degrees F.  
They are then pulled from the fire. These oils  
may undergo an automatic rise in temperature  
thereafter beyond 480 degrees F., but this is un-  
necessary and too great a rise should be avoided. 15

When the temperature of these oils has started  
to drop reaching approximately 475 degrees F., we add 3 1/2 pounds of litharge, stirring until the  
litharge is taken up by the oil. The temperature  
of this batch is then run back and forth between 20  
460 degrees and 470 degrees, being held within  
this range for approximately 30 minutes and in  
some cases a little longer until sufficient body  
has been imparted to the oil and litharge.

Thereafter we add 8 1/2 pounds of manganese 25  
solid linoleate and 2 pounds of cobalt solid lino-  
leate. These soluble driers melt into the batch.

We then add 67 pounds of synthetic resin solid,  
known to the trade as "Amberol B/S 1 Light." 30  
This is melted at a low heat. Then the tempera-  
ture is carried back to approximately 425 de-  
grees F.

We then thin the batch at once with 14 gal-  
lons each of heavy and light petroleum naphtha.

The resulting compound may be used by itself 35  
or in combination with the product of the formula  
hereinafter recited.

Thereafter we prepare Varnish B.

40 Varnish B

This formula is as follows:

|                      | Pounds |
|----------------------|--------|
| South sea gum (Batu) | 67     |
| Litharge             | 3 1/2  |
| Managanese linoleate | 8 1/2  |
| Cobalt linoleate     | 2      |

|                         | Gallons |
|-------------------------|---------|
| China-wood oil          | 20      |
| Linseed oil             | 2 1/4   |
| Heavy petroleum naphtha | 20      |
| Light petroleum naphtha | 20      |

The cooking is carried out in this manner.  
Sixty-seven pounds of South Sea gum, also known 55

*Drier example*

One of the preferred formulas which we have used is as follows:

|                        | Pounds |
|------------------------|--------|
| Linoleate of lead      | 385    |
| Linoleate of cobalt    | 889    |
| Linoleate of manganese | 14     |

These are melted at as low heat as possible, and when entirely fluid the mass is thinned with 10 1202 gallons of turpentine, either gum spirits or wood spirits, or some slowly evaporating coal tar fraction, such as xylene. It will be understood that the proportions of these elements of the drier can be varied according to the result desired. By adjusting these proportions the velocity of the surface drying and drying throughout the film can be regulated.

It will be understood that we desire to comprehend within our invention such modifications 20 as come within the scope of our claims and our invention.

Having thus fully described our invention, what we claim as new and desire to secure by Letters 25 Patent, is:

1. In an improved enamel composition for producing imitation leather finishes which are air-drying at temperatures between 60 and 90 degrees F., a synthetic resin varnish, a natural resin varnish in the proportions of from two to 30 one or one to two parts with respect to one another, raw China-wood oil in the proportion of from five to twenty-five parts, and a drier in the proportion of from five to twenty-five parts, said drier consisting of linoleates of cobalt, lead and 35 manganese.

2. In an improved enamel composition for producing imitation leather finishes which are air-drying between 60 and 90 degrees F., a synthetic resin varnish, a natural resin varnish in the proportions of from two to one or one to two parts with respect to one another, raw China-wood oil in the proportion of from five to twenty-five parts, a drier, consisting of linoleates of cobalt, 40 lead and manganese, in the proportion of from five to twenty-five parts, and from one to ten parts of a petroleum naphtha thinner.

3. In an improved enamel composition for producing imitation leather finishes which are air-drying between 60 and 90 degrees F., a synthetic resin varnish, a natural resin varnish in the proportions of from two to one or one to two parts with respect to one another, raw China-wood oil in the proportion of from five to twenty-five parts, a drier, consisting of linoleates of cobalt, 45 lead and manganese, in the proportion of from five to twenty-five parts, and from one to ten parts of a petroleum naphtha thinner, said drier comprising linoleate of lead, linoleate of cobalt, 50 linoleate of manganese, and a solvent.

4. In an improved enamel composition for producing imitation leather finishes which are air-drying at temperatures between 60 and 90 degrees F., approximately eighty-one parts of synthetic resin varnish, approximately forty and one-half parts of natural resin varnish, approximately nine parts of raw China-wood oil, approximately nine parts of a drier composed of linoleate of lead, 55 linoleate of cobalt and linoleate of manganese 60 mixed with turpentine, and one to ten parts of petroleum naphtha thinner.

5. In an improved enamel composition for producing imitation leather finishes which are air-drying at temperatures approximating nor-

as Batu gum, are run in the ordinary approved fashion customary in varnish making. Then 20 gallons of China-wood oil and 2 1/4 gallons of refined linseed oil are mixed and heated slowly until they reach 300 or 350 degrees F., then they are added slowly to the gum when the latter has been well run.

The mixture is then carried to a temperature of 460 to 470 degrees F. and held within this 10 range, in order to impart body to the mixture, for about 30 minutes or a little longer.

We then stir into the batch 3 1/2 pounds of litharge until it is taken up and fully incorporated in the batch. The 8 1/2 pounds of manganese solid linoleate and 2 pounds of cobalt solid linoleate are allowed to melt in the batch.

We then thin at once with 20 gallons each of heavy and light petroleum naphtha. Turpentine may be substituted for the naphtha.

20 In order to make the compound of this invention, either one of the above varnishes or both are combined with raw tung (China-wood) oil and a drier. A thinner can be added optionally. The proportion of Varnish A with respect to Varnish B may be two to one, or vary therebetween, or Varnish B with respect to Varnish A may be two to one, or vary therebetween. In either event, the China-wood oil will vary in number of parts from approximately 5 to 25 parts. The 30 drier will vary from approximately 5 to 25 parts, and the thinner will vary from 1 to 10 parts, depending upon the viscosity desired.

*Example 1*

35 A typical example of a satisfactory compound for the practice of this invention is the following:

|                           | Parts  |
|---------------------------|--------|
| 40 Varnish A              | 81     |
| Varnish B                 | 40 1/2 |
| Raw tung (China-wood) oil | 9      |
| Drier                     | 9      |
| Petroleum naphtha         | 5-10   |

45 To one gallon of this compound we add 5 to 7 pounds of the desired color, previously ground in spar varnish.

Varnish A has the function of fast drying, and 50 imparts a high luster. Varnish B has a medium drying rate, and provides a low luster. China-wood oil facilitates a very wrinkled drying without gloss and adds opacity to the product. The thinner controls the viscosity and the drier has the following functions and characteristics:

55 When the compound of this invention is applied it must first flow out evenly on the surface treated and then the drying must begin almost at once on the surface of the wet compound by the formation of microscopic wrinkles. This initial wrinkling then proceeds through the whole thickness of the film as the complete drying 60 proceeds.

The preferred drier that we have found to 65 best serve this purpose comprises linoleate of lead, linoleate of cobalt, and linoleate of manganese. The cobalt and manganese, particularly the cobalt, accelerate the surface drying, as described above, while the lead and manganese are utilized for completing the drying completely 70 through the film. This combination of cobalt and manganese supplies quick initial surface drying necessary, while the lead and the manganese supply the necessary catalytic action for the drying through the film.

5 mal room temperature, approximately eighty-one parts of synthetic resin varnish, approximately forty and one-half parts of natural resin varnish, approximately nine parts of raw China-wood oil, approximately nine parts of a drier composed of linoleate of lead, linoleate of cobalt and linoleate of manganese mixed with turpentine, one to ten parts of petroleum naphtha thinner, and a color compound ground in spar  
10 varnish.

10 6. In an improved enamel composition for producing imitation leather finishes which are air-drying at temperatures between 60 and 70 degrees F., the combination of the following: Approximately eighty-one parts of synthetic resin Varnish A; approximately forty and one-half parts Varnish B; approximately nine parts of raw China-wood oil; approximately nine parts of a drier composed of linoleate of lead, linoleate of cobalt and linoleate of manganese, and turpentine solvent, 15  
20

7. In an improved enamel composition for producing imitation leather finishes which are air-drying at temperatures between 60 and 70 degrees

F., the combination of the following: Approximately eighty-one parts of synthetic resin Varnish A; approximately forty and one-half parts Varnish B; approximately nine parts of raw China-wood oil; approximately nine parts of a drier composed of linoleate of lead, linoleate of cobalt and linoleate of manganese, turpentine solvent, and from one to ten parts of petroleum naphtha. 5

8. In an improved enamel composition for producing imitation leather finishes which are air-drying between 60 and 80 degrees F., the combination of the following: Approximately eighty-one parts of synthetic resin Varnish A; approximately forty and one-half parts Varnish B; approximately nine parts of raw China-wood oil; approximately nine parts of a drier composed of linoleate of lead, linoleate of cobalt and linoleate of manganese, turpentine solvent, from one to ten parts of petroleum naphtha, and a color 15  
20 ground in spar varnish.

HARVEY G. KITTREDGE.  
ALBERT J. TURNER.